

1

3,099,545

**BUFFING WHEEL**

Richard S. Johnson, 1032 S. 42nd St., Birmingham 5, Ala.  
No Drawing. Filed Feb. 1, 1961, Ser. No. 86,319  
2 Claims. (Cl. 51—298)

This invention relates to buffing wheels made from textile fabrics, and more particularly to buffing wheels that have been treated with a resinous composition.

The buffing wheel of the present invention is particularly characterized in its excellence for buffing aluminum and aluminum alloys.

Some of the prior art buffing wheels that have been dipped in various resinous compositions are characterized in that the composition causes the fabric of the buffing wheel to become brittle and to break off when the buffing wheel is repeatedly flexed during the buffing operation. This results in a short wheel life, and more importantly these broken bits of coated fabric become part of an excessive head that develops during the buffing operation. This head is a combination of elements that builds upon and coats the outer periphery of the buffing wheel during the buffing operation; it is composed of metallic particles from the article being buffed, bits of frayed fabric from the buffing wheel, granules of abrasive dust supplied during the buffing operation and waxes, tallows and oils from the vehicle carrying the abrasive dust. This excessive head build up, or accumulation of elements, which is characteristic of all prior art buffing wheels, interferes with the approach of the buffing wheel fabric and the abrasive to the metal being buffed, thus causing inefficiency in the buffing operation. A further disadvantage is that the excessive head causes scratching, tearing and marking off of the metal being buffed, especially in the case of aluminum and aluminum alloys because of their relatively soft character, thus defeating the purpose of the buffing operation, which is the removal of scratches and the production of a smooth surface upon the metal being buffed.

Another and further disadvantage of the dipped buffing wheels of the prior art is excessive fraying of the fabric forming the outer periphery of the buffing wheel, which also causes excessive head build up and short wheel life.

The problems listed above have been solved by the present invention which comprises treating the cotton buffing wheel with a resinous composition, particularly a modified alkyd resin, a mixture of a rosin derivative, a plasticizer and a suitable solvent. The buffing wheel is dipped into the composition, thus impregnating the fabric, coating the yarns and fibers, and cementing the adjacent yarns together. In this manner, the cemented yarns are bound together and become stronger, with greatly reduced fiber breakage. Also, fraying of the fabric on the outer periphery of the buffing wheel is markedly reduced. Since the head build up can only become as thick as the depth of the frayed fabric as measured on the radius of the wheel, the depth of head is correspondingly minimized as the frayed fabric area is reduced. This decrease of the head results in an increased area of contact between the metal being buffed, the buffing wheel fabric and the abrasive that is utilized in buffing, thus resulting in increased buffing efficiency. The lessening of fiber breakage causes fewer bits of broken fabric to be contributed to the head composition, thus further reducing the head build up. Since the above head is made smaller, fewer metallic particles from the article being buffed may accumulate on the head, resulting in less scratching, tearing and marking off of the metal being buffed.

Although prior resinous compositions have to some extent cemented together the adjacent yarns of buffing wheels, none has produced a cotton buffing wheel as efficient as may be done by the present invention.

Although the foregoing discussion has been directed to

2

cotton buffing wheels, it will be realized that the present invention is not limited to buffing wheels made from cotton fabric, but also contemplates buffing wheels made from other textile fabrics and arrangements of fibers, both natural and synthetic.

The following are examples of the present invention:

*Example I*

A resinous composition is made according to the following formula, all parts by weight:

| Component:                                                                                                                                                                                                                                              | Percent by weight |
|---------------------------------------------------------------------------------------------------------------------------------------------------------------------------------------------------------------------------------------------------------|-------------------|
| Pentaerythritol ester of modified rosin (the product obtained by the substantially complete esterification, with pentaerythritol, of the rosin acids present in rosin that has been modified by the formation of an adduct with maleic anhydride) ----- | 15                |
| Styrenated alkyd resin (the product obtained from the interpolymerization of monomeric styrene with the polymer formed from a soya bean oil modified glycerol ester of phthalic and maleic anhydride, containing 50% reacted styrene) -----             | 15                |
| Toluene -----                                                                                                                                                                                                                                           | 60                |
| Castor oil -----                                                                                                                                                                                                                                        | 10                |
| Total -----                                                                                                                                                                                                                                             | 100               |

All of the operations are carried out at room temperature, and the composition need not be compounded in any particular order. The composition is stable over a long period of time.

A pre-formed conventional cotton fabric buffing wheel is totally immersed into a vat containing the above composition at room temperature for thirty seconds, and an amount of solution equal to about 25-30% of the weight of the fabric is taken up by the fabric. The buffing wheel is then removed from the mixture and rotated for thirty seconds upon its axis on the same plane and at the same speed at which the wheel will later be operated, for example 1,000-3,000 r.p.m., depending on the diameter of the wheel. The remaining solvent is then evaporated in a current of air until the buffing wheel is substantially dry.

*Example II*

A resinous composition is made according to the formula disclosed in Example I, above.

A pre-formed conventional sisal fabric buffing wheel is totally immersed into a vat containing the above composition at room temperature for thirty seconds, and an amount of solution equal to about 25-30% of the weight of the fabric is taken up by the fabric. The buffing wheel is then removed from the mixture and rotated for thirty seconds upon its axis on the same plane and at the same speed at which the wheel will later be operated, for example 1,000-3,000 r.p.m., depending on the diameter of the wheel. The remaining solvent is then evaporated in a current of air until the buffing wheel is substantially dry.

It is preferred that the buffing wheel be rotated in the above mentioned manner so that the resinous composition will be evenly deposited over the wheel and a dynamically balanced wheel be produced, although it is not essential. Unbalanced buffing wheels will cause excessive wearing of the bearings and journals of buffing machinery.

Advantageous results have been obtained from the above described pentaerythritol ester of modified rosin, but it is contemplated that rosin modified phenolic resins, the pentaerythritol ester of rosin, the modified rosin sold under the trade name "Pentacite 1405" by Reichhold Chemicals, Inc., or the modified rosin sold under the trade name "Pentalyn 860" by Hercules Powder Company may be

substituted therefor. Likewise, the above described styrenated alkyd resin is utilized as the preferred modifier. However, the styrenated alkyd polymer of other oil modified alkyd resins, such as those obtained from reacting castor oil with glycerol and a mixture of phthalic and maleic anhydrides or phthalic anhydride and fumaric acid, or the resin sold under the trade name "Styresol 4250" by Reichhold Chemicals, Inc., may be substituted therefor. Further, it is desirable that the oil used in modifying the resin be a non-drying oil rather than a drying oil, because of the inherent danger of spontaneous combustion in using chemical compounds derived from drying oils in textile fabrics.

In addition, the resin should contain 20-60% by weight of reacted styrene and should be chosen from the group of styrenated oil modified alkyd resins that, when cast into thin sheets or films, display superior abrasion resistance and heat stability. Toluene is utilized as the preferred solvent for the solid components in the present invention, because it has the advantage of relatively low toxicity, intermediate evaporation rate, and because of its aromatic character. However, it is contemplated that a xylene-toluene mixture or benzene may be substituted therefor. Castor oil is utilized as the preferred plasticizer, but it is contemplated that dioctyl phthalate, or tris(2,3 dichloropropyl) orthophosphate may be substituted therefor. This latter plasticizer imparts excellent flame retardant properties to the buffing wheel.

While the preferred embodiment of the invention and the preferred manner of practicing the present method have been described, it will be understood that the invention may be embodied in other forms and applied to other methods within the scope of the following claims.

I claim:

- As a new article of manufacture, a buffing wheel made of cotton textile fabric that has been treated with a composition comprising 15% of a member selected from the group consisting of pentaerythritol ester of modified rosin, rosin modified phenolic resin, pentaerythritol ester of rosin, and modified rosin, 15% of a member selected from the group consisting of styrenated alkyd resin and styrenated alkyd polymer of oil modified alkyd resin, 60% of a solvent selected from the group consisting of toluene, benzene, and xylene-toluene mixture, and 10% of a plasticizer selected from the group consisting of castor oil, dioctyl phthalate, and tris (2,3 dichloropropyl) orthophosphate and thereafter dried.
- As a new article of manufacture, a buffing wheel made of sisal textile fabric that has been treated with a composition comprising 15% of a member selected from the group consisting of pentaerythritol ester of modified rosin, rosin modified phenolic resin, pentaerythritol ester of rosin, and modified rosin, 15% of a member selected from the group consisting of styrenated alkyd resin and styrenated alkyd polymer of oil modified alkyd resin, 60% of a solvent selected from the group consisting of toluene, benzene, and xylene-toluene mixture, and 10% of a plasticizer selected from the group consisting of castor oil, dioctyl phthalate, and tris (2,3 dichloropropyl) orthophosphate and thereafter dried.

**References Cited in the file of this patent**

**UNITED STATES PATENTS**

- |           |                         |               |
|-----------|-------------------------|---------------|
| 2,060,665 | Durant et al. -----     | Nov. 10, 1936 |
| 2,851,379 | Staudinger et al. ----- | Sept. 9, 1958 |
| 2,890,137 | Vaughan et al. -----    | June 9, 1959  |

UNITED STATES PATENT OFFICE  
CERTIFICATE OF CORRECTION

Patent No. 3,099,545

July 30, 1963

Richard S. Johnson

It is hereby certified that error appears in the above numbered patent requiring correction and that the said Letters Patent should read as corrected below.

In the grant, lines 1 to 3, for "Richard S. Johnson, of Birmingham, Alabama," read -- Richard S. Johnson, of Birmingham, Alabama, assignor, by mesne assignments, to Jackson Buff Corporation, of Conover, North Carolina, a corporation of North Carolina, --; line 12, for "Richard S. Johnson, his heirs" read -- Jackson Buff Corporation, its successors --; in the heading to the printed specification, line 3, for "Richard S. Johnson, 1032 S. 42nd St., Birmingham 5, Ala." read -- Richard S. Johnson, Birmingham, Ala., assignor, by mesne assignments, to Jackson Buff Corporation, Conover, N. C., a corporation of North Carolina --; column 1, line 43, for "has" read -- have --; column 2, line 22, for "anhydride" read -- anhydrides --; line 49, for "containg" read -- containing --.

Signed and sealed this 12th day of May 1964.

(SEAL)  
Attest:

ERNEST W. SWIDER

Attesting Officer

EDWARD J. BRENNER

Commissioner of Patents